

1

2,913,407

TEXTILE LUBRICANTS

Knapel F. Schiermeier, Alton, Ill., assignor to Shell Development Company, New York, N.Y., a corporation of Delaware

No Drawing. Application July 29, 1957  
Serial No. 674,557

5 Claims. (Cl. 252—8.7)

This invention relates to textile lubricants for processing synthetic fibers such as nylon and the like. More particularly, this invention is directed to mineral oil compositions, for use in processing nylon fibers, which are stable, non-corrosive, prevent staining and size build-up, and which possess good scourability properties.

It is common practice in the art to use as textile lubricants for natural fibers such as wool, cotton, silk and the like as well as some synthetics such as rayons or cellulose nitrates, mineral oils containing small amounts of soaps or sulfonates or mixtures of soaps and fats, fatty acids and esters thereof or esters of polyhydric alcohols and long-chain fatty acids and alkylene oxide derivatives thereof and the like. Such textile lubricants are generally suitable for processing fibers of the above types. However, they have been found to be poor for processing nylon fibers due to their tendency to cause staining, size build-up and their poor scourability properties. Also, such lubricants tend to form gummy deposits on machinery surfaces, and cause corrosion particularly of non-ferrous metals such as brass and copper.

It is a principal object of this invention to prepare an inexpensive and improved textile lubricant particularly applicable for processing of synthetic fibers such as nylon. Another object of this invention is to prepare a stable, non-corrosive nylon textile mineral oil base lubricant which is resistant to size build-up, staining and which possesses good scourability.

It has now been discovered that an excellent textile lubricant, particularly suitable for processing nylon, is provided by a highly refined light mineral oil containing an additive combination, in critical amounts, of from about 0.25% to about 3%, preferably from about 0.5% to 2.5%, each of (1) an oil-soluble alkali metal (e.g. Na or K) petroleum sulfonate, (2) a partial ester derived from simple alkanepolyols and fatty acids of at least 12, preferably 14-18 carbon atoms, (3) a mixture of (a) from 60% to 90% of an ester of a monohydric aliphatic alcohol of from 3 to 8 carbon atoms and a fatty acid of from 1 to 5 carbon atoms and (b) from 10% to 30% of a free alcohol of the same class and (4) an oil-soluble alkyl phenol.

The oil-soluble alkali metal petroleum sulfonates are well known in the art and are prepared by reacting a mineral oil with concentrated or fuming sulfuric acid to form oil-soluble sulfonic acids which are then recovered by treatment with an alkali metal base such as sodium hydroxide followed by extraction. These oil-soluble soaps are available as 30% to 70% concentrates in mineral oil and are used preferably in an amount of 0.5 to 1.5% by weight.

The second essential additive is a partial ester of a simple alkanepolyol and a C<sub>12-18</sub> saturated or unsaturated fatty acid. The alkanepolyols include alkylene glycols e.g. ethylene or propylene glycol, glycerol, erythritol, pentaerythritol, sorbitol, mannitol and the like. The acids which can be used to make the partial esters from

2

any of the above alcohols include saturated and unsaturated fatty acids of from 12 to 18 carbon atoms, such as lauric, myristic, stearic, oleic, linoleic and ricinoleic acids. These partial esters are preferably used in an amount of from 1 to 2.5% by weight.

Specific esters derived from simple alkanepolyols and long chain fatty acids include glycerol monooleate, glycerol monostearate, glycerol monoricinoleate, pentaerythritol mono- and dilaurate, pentaerythritol mono- and dioleate, pentaerythritol mono- and distearate, mono-, di-, and triethylene glycol monooleate, propylene glycol monoricinoleate, ethylene glycol monooleate, triethylene glycol monostearate, sorbitol monolaurate, mannitol monooleate, mannitol dioleate, sorbitol dioleate, etc.

The third essential additive is a material which is a blend or mixture of an ester of a monohydric aliphatic alcohol of from 2 to 8 carbon atoms and a fatty acid of from 1 to 5 carbon atoms and an alcohol including the normal and branched-chain alcohols having from 2 to 8 carbon atoms such as ethyl, propyl, butyl, amyl, hexyl, octyl, isopropyl, isobutyl, isoamyl or iso-octyl alcohols.

The acids used to make the esters include fatty acids of from 1 to 5 carbon atoms such as formic, acetic, propionic, butyric, isobutyric or valeric acids. Specific examples of esters of this class include, propyl acetate, iso-

propyl acetate, butyl acetate, butyl propionate, isobutyl acetate, amyl acetate, isoamyl acetate, amyl butyrate, amyl valerate, and the like. Specific examples of the ester-alcohol mixture in amount indicated above include iso-

propyl acetate-isopropyl alcohol, butyl acetate-butyl alcohol, isobutyl acetate-isobutyl alcohol, amyl acetate-amyl alcohol, isoamyl acetate-isoamyl alcohol and mixtures thereof. The ester-alcohol mixture is preferably used in an amount of 0.5 to 2% by weight.

The fourth essential additive is an oil-soluble alkyl phenol e.g. di- and trialkyl phenols, for instance 2,4-, 2,3-, 2,6- and 3,5-diamyl or dihexyl phenol, 2,4-dimethyl-6-tert-butyl phenol, 2,6-ditert-butyl-4-methyl phenol and mixtures thereof. These alkylphenols are preferably employed in an amount of 0.25 to 0.5% by weight.

The liquid mineral oil is a light petroleum hydrocarbon fraction in the viscosity range of from about 40 to about 200 SUS at 100° F., preferably from about 60 to about 120 SUS at 100° F. Petroleum fractions of this type

can be derived from any type of crude such as asphaltic, naphthenic or paraffinic type crudes. It is preferred to use a refined light lubricating oil such as a selective solvent-refined raffinate having a viscosity of 100 SUS at 100° F.

The following examples illustrate compositions of this invention. The mineral oil in such example was a raffinate obtained by a phenol extraction, using West Texas Ellenburger base stock.

EXAMPLE I

|                                                | Percent weight |
|------------------------------------------------|----------------|
| Sodium petroleum sulfonate (oil-soluble)       | 0.5            |
| Glycerol monooleate                            | 2.25           |
| Mixture of isomeric amyl acetates and amyl al- |                |
| cohols (ester content 85% by wt.)              | 1.50           |
| 2,6-ditert-butyl-4-methyl phenol               | 0.5            |
| Mineral oil (100 SUS at 100° F.)               | Balance        |

EXAMPLE II

|                                                | Percent weight |
|------------------------------------------------|----------------|
| Potassium petroleum sulfonate (oil-soluble)    | 0.5            |
| Glycerol monooleate                            | 2.25           |
| Mixture of isomeric amyl acetates and amyl al- |                |
| cohols (ester content 85%)                     | 1.50           |
| 2,6-ditert-butyl-4-methyl phenol               | 0.5            |
| Mineral oil (100 SUS at 100° F.)               | Balance        |

## EXAMPLE III

|                                                                         | Percent weight |
|-------------------------------------------------------------------------|----------------|
| Sodium petroleum sulfonate (oil-soluble)                                | 0.5            |
| Pentaerythritol monooleate                                              | 2.25           |
| Mixture of isomeric amyl acetates and amyl alcohols (ester content 85%) | 1.50           |
| 2,6-ditert-butyl-4-methyl phenol                                        | 0.5            |
| Mineral oil (100 SUS at 100° F.)                                        | Balance        |

## EXAMPLE IV

|                                                | Percent weight |
|------------------------------------------------|----------------|
| Sodium petroleum sulfonate (oil-soluble)       | 0.25           |
| Glycerol monooleate                            | 1.2            |
| Amyl acetate-amyl alcohol mixture (85% esters) | 0.75           |
| 2,6-ditert-butyl-4-methyl phenol               | 0.25           |
| Mineral oil (100 SUS at 100° F.)               | Balance        |

## EXAMPLE V

|                                                    | Percent weight |
|----------------------------------------------------|----------------|
| Sodium petroleum sulfonate (oil-soluble)           | 1.0            |
| Glycerol monostearate                              | 2.0            |
| Mixture of butyl acetate-butyl alcohol (67% ester) | 1.0            |
| 2,4 diamyl phenol                                  | 0.25           |
| Mineral oil (150 SUS at 100° F.)                   | Balance        |

Compositions of the present invention were compared with a number of textile oils including a commercial textile oil (Composition A) for stability (Dornte oxidation test and storage stability), corrosion toward brass and copper at 212° F., scourability, size build-up and staining while processing nylon and the results are shown in Table I.

Table I

| Composition                | Dornte Oxidation (250° F., min.) | Storage Stability (Room Temp.) | Scourability | Staining of fiber | Size Build Up | On and Brass Corrosion |
|----------------------------|----------------------------------|--------------------------------|--------------|-------------------|---------------|------------------------|
| Example I                  | 1,680                            | 1 month (excellent)            | Excellent    | None (nylon)      | None          | None                   |
| Composition A <sup>1</sup> | 480                              | do                             | Poor         | Heavy             | Heavy         | Heavy                  |
| Composition B <sup>2</sup> | 275                              | 1 month (rancid)               | do           | do                | do            | Do                     |
| Composition C <sup>3</sup> | 1,000                            | 1 month (good)                 | do           | Medium            | do            | None                   |

<sup>1</sup> Composition A—commercial textile oil comprising a mineral oil containing a soap, fatty oil, fatty acid and a sulfonated vegetable oil.

<sup>2</sup> Composition B—mineral oil containing 10% lard oil.

<sup>3</sup> Composition C—mineral oil containing 0.5% Na petroleum sulfonate+2% glycerol monooleate.

Compositions of Examples II to V when subjected to the above tests gave comparable results to the composition of Example I.

Example I was used as a needle oil in a mill machine making nylon seamless hose. The machine was in excellent condition and no size build-up occurred after months of operation. However, when an oil composition D (mineral oil+0.5% Na petroleum sulfonate+2.25% glycerol monooleate+0.5% 2,6 ditert-butyl-4-methyl phenol) similar to Example I was used as a needle oil, but from which the amyl acetate-amyl alcohol mixture was omitted considerable staining and size build-up occurred and the operations had to be stopped after a few days.

I claim as my invention:

1. A textile lubricating composition consisting essentially of a major amount of mineral oil containing from about 0.25% to about 3% each of (1) an oil-soluble alkali metal petroleum sulfonate, (2) a partial ester of a simple alkanopolyol and a fatty acid having from 12 to 18 carbon atoms, (3) a mixture of (a) an ester of a monohydric aliphatic alcohol having from 2 to 8 carbon atoms and a fatty acid having from 1 to 5 carbon atoms and (b) a monohydric aliphatic alcohol having from 2

to 8 carbon atoms portion (a) being 60-90% and portion (b) being 10-30% of mixture (3) and (4) an alkyl phenol.

2. A textile lubricating composition for knitting of nylon fibers, consisting essentially of a major amount of mineral oil containing from about 0.25% to about 3% each of (1) oil-soluble sodium petroleum sulfonate, (2) a partial ester of glycerol and a fatty acid having from 12 to 18 carbon atoms, (3) a mixture of (a) esters of an amyl alcohol and a fatty acid having from 1 to 5 carbon atoms and (b) amyl alcohols the ester portion of the mixture being 60-90% and the alcohol portion of the mixture being 10-30% and a polyalkyl phenol.

3. A textile lubricating composition for knitting of nylon fibers, consisting essentially of a major amount of mineral oil containing from about 0.25% to about 3% each of (1) oil-soluble sodium petroleum sulfonate, (2) glycerol monooleate, (3) mixture of amyl acetates and amyl alcohols the ester portion of the mixture being 60-90% and the alcohol portion of the mixture being 10-30% and (4) 2,6 ditert-butyl-4-methyl phenol.

4. A textile lubricating composition for knitting of nylon fibers, consisting essentially of a major amount of mineral oil containing from about 0.25% to about 3% each of (1) oil-soluble potassium petroleum sulfonate, (2) glycerol monooleate, (3) mixture of amyl acetates and amyl alcohols the ester portion of the mixture being 60-90% and the alcohol portion of the mixture being 10-30% and (4) 2,6 ditert-butyl-4-methyl phenol.

5. A nylon textile lubricating composition having the formula by weight:

|                                                                 | Percent |
|-----------------------------------------------------------------|---------|
| Oil-soluble sodium petroleum sulfonate                          | 0.5     |
| Glycerol monooleate                                             | 2.25    |
| Mixture of isomeric amyl acetates (85%) and amyl alcohols (15%) | 1.50    |
| 2,6 ditert-butyl-4-methyl phenol                                | 0.5     |
| Mineral oil                                                     | Balance |

## 55 References Cited in the file of this patent

## UNITED STATES PATENTS

|           |             |               |
|-----------|-------------|---------------|
| 2,575,382 | Duke et al. | Nov. 20, 1951 |
| 2,644,766 | Levine      | July 7, 1953  |
| 2,730,464 | Winsor      | Jan. 10, 1956 |
| 2,807,864 | Head        | Oct. 1, 1957  |
| 2,810,694 | McLean      | Oct. 22, 1957 |

## OTHER REFERENCES

65 "Phenolic Antioxidants for Paraffinic Materials," article by Morawetz, Ind. Eng. Chem., July 1949, pp. 1442-46.